

# UNITED STATES PATENT OFFICE.

CHRISTIAN EMIL BICHEL, OF HAMBURG, GERMANY.

## EXPLOSIVE.

No. 887,027.

Specification of Letters Patent.

Patented May 5, 1908.

Original application filed July 6, 1903, Serial No. 164,453. Divided and this application filed May 24, 1905.  
Serial No. 262,089.

*To all whom it may concern:*

Be it known that I, CHRISTIAN EMIL BICHEL, a subject of the German Emperor, residing at Hamburg, in the German Empire, 5 have invented certain new and useful Improvements in Explosives; and I do hereby declare the following to be a full, clear, and exact description of the invention, such as will enable others skilled in the art to which 10 it appertains to make and use the same.

My invention relates to fire-damp proof explosives, which are short flamed and quick burning, but more particularly to means for further dampening the flame of such explosives 15 to render them safer and less liable to ignite fire-damp and so that they will not exert an injurious effect on the choke-damps, *i. e.*, so that the products of explosion will not injuriously affect the air in the mine to 20 pleasantly affect the breathing of the workmen; this application being a division of my application Serial Number 164,453, filed July 6, 1903.

I have found that the addition of an alkaline metal chlorid will dampen the flame of short flame and quick burning explosives and prevent them from igniting fire-damp as well as coal dust laden atmospheres of mines. This I accomplish by incorporating in the explosive such salts as will by double decomposition produce the desired alkaline metal chlorid, the vapor of which is not deleterious to health and does not contaminate the air in the mine to make it unpleasant to breathe. 30 These salts are used, preferably, but not necessarily, in equivalent quantities, that is, quantities such that the desired elements will be present to recombine to form the required quantity of alkaline metal chlorid. To this 35 end I add to the explosive or incorporate in it a nitrate of an alkaline metal, such as sodium or potassium nitrate and a suitable chlorid as ammonium chlorid, which by the combustion of the explosive form alkaline metal chlorid.

It has been stated by official commissions in countries where fiery mines are worked, that all explosives when fired in mixtures of pit gas or coal-dust are liable to ignite this mixture if the quantity used for the shot is 45 large enough.

It is the object of this invention to render most of the explosives safer against fire-

damp and dry coal-dust, than they are without the means mentioned herein. For example, the quantity of usual No. 1 dynamite (of 75% nitroglycerin and 25% of kieselguhr) of 5 grams regularly ignites a mixture of 8% of fire-damp (or a suitable quantity of benzine vapor which gives the same effect), whereas an explosive manufactured in accordance with this invention requires a quantity of more than 500 grams without losing a great percentage of its strength, so that the safety is as 5 is to 500. The object of the invention therefore is to render the work in 55 60 65 fiery mines safer.

The examples given hereinafter, recording, as they do, the results of actual experience, will confirm the above statements and the success of the invention.

### 1. Donarite of the following compositions:

|                    |     |           |
|--------------------|-----|-----------|
| Nitrate of ammonia | 80  | per cent. |
| Trinitrotoluol     | 12  | " "       |
| Flour              | 4   | " "       |
| Nitroglycerin      | 3.8 | " "       |
| Collodion-cotton   | 0.2 | " "       |

#### *Safety:*

|                                                                                               |     |       |
|-----------------------------------------------------------------------------------------------|-----|-------|
| Donarite alone                                                                                | 87  | grams |
| 95 per cent. of donarite + 5 per cent. ammonium chlorid                                       | 125 | "     |
| 90 per cent. of donarite + 10 per cent. of ammonium chlorid                                   | 250 | "     |
| 86 per cent. of donarite + 5.5 per cent. of ammonium chlorid and 8.5 per cent. sodium nitrate | 425 | "     |

There was a reduction in the power displayed amounting to about 8 per cent., while safety was enhanced five-fold.

### 2. Roburite of the following composition:

|                           |      |           |
|---------------------------|------|-----------|
| Nitrate of ammonia        | 72.5 | per cent. |
| Binitrobenzol             | 12   | " "       |
| Potassium nitrate         | 10   | " "       |
| Sulfate of ammonium       | 5    | " "       |
| Permanganate of potassium | 0.5  | " "       |

#### *Safety:*

|                                                                 |     |       |
|-----------------------------------------------------------------|-----|-------|
| Roburite alone                                                  | 325 | grams |
| Roburite with ammonium chlorid substituted for ammonium sulfate | 100 | "     |
|                                                                 | 400 | "     |

At the same time there occurred an increase in the power.

3. An explosive hereinafter termed X, of the following composition:

|                    |      |           |
|--------------------|------|-----------|
| Nitroglycerin      | 4    | per cent. |
| Nitrate of ammonia | 75.5 | " "       |
| Potassium nitrate  | 9.5  | " "       |
| Coal dust          | 0.5  | " "       |
| Flour              | 10.5 | " "       |

*Safety:*

|    |                               |     |       |
|----|-------------------------------|-----|-------|
| 10 | Explosive X alone             | 250 | grams |
| 95 | per cent. of explosive X+5    |     |       |
| 92 | percent. of ammonium chlorid  | 400 | "     |
| 15 | 92 per cent. of explosive X+8 |     |       |
|    | percent. of ammonium chlorid  | 500 | "     |

The power displayed became reduced by 3 per cent. when 5 per cent. of ammonium chlorid was added to the explosive.

The following table is intended to account for the influence exerted by ammonium chlorid when added to explosive X, the explosive of the aforesaid composition, viz:

| 25                                                                | Heat evolved at explosion, at thermal units. | Duration of flame (or flash) in 1/1000 of a second. | Length of flame in centimeters | Safety in grams. |
|-------------------------------------------------------------------|----------------------------------------------|-----------------------------------------------------|--------------------------------|------------------|
| Explosive X alone 863.....                                        | 0.403                                        | 54                                                  | 250                            |                  |
| 95 per cent. explosive X+8 per cent. ammonium chlorid 781.....    | 0.262                                        | 45                                                  | 400                            |                  |
| 30 92 per cent. explosive X+8 per cent. ammonium chlorid 745..... | 0.210                                        | 40                                                  | 500 and upwards.               |                  |

This table is based upon the method of investigation of explosives published in part III Vol. 50 of the journal *Zeitschrift für Berg-, Hütten- und Salinenwesen*.

Hence it will be seen that by the addition of ammonium chlorid to the explosive X already containing 9.5 per cent. of potassium nitrate the number of thermal units, the time of flash, and the length of flame are reduced, while the safety from fire-damp is made to become double what it was before, that is to say, without the separate addition of ammonium chlorid.

By incorporating in or adding to the explosive or blasting powder a nitrate of an alkaline metal and a suitable chlorid, I accomplish two things, first, the acid radical of the nitrate will furnish oxygen for the combustion and its metallic radical will combine with the chlorin of the chlorid to produce a dampener for the flame.

I wish it understood that in the claims, the term alkaline metal salt means not only a single salt of such, but also a mixture of such salts and although I mention a single chlorid, mixtures of chlorids are to be also intended, since it is immaterial whether a single salt, as a nitrate and a chlorid or mixtures of nitrates and chlorids of different metals are used, the primary object being to form as one

of the products of the explosion, the vapor of a chlorid of an alkaline metal or metals, such as sodium chlorid, potassium chlorid or both.

Having thus described my invention, what I claim as new therein and desire to secure by Letters Patent, is:

1. A short flame detonating explosive containing a salt of an alkaline metal and a suitable chlorid intimately mixed, which by double decomposition, on explosion will produce vapor of an alkaline metal chlorid sufficient to damp the flame and thereby prevent ignition and explosion of fire-damp, substantially as described.

2. A short flame, detonating explosive containing substantially combining weights of chlorid of ammonium and a nitrate of an alkaline metal intimately mixed to produce an inert product of combustion sufficient to damp the flame and enhance the safety of the explosive against fire-damp explosions, substantially as described.

3. A short flame detonating explosive containing chlorid of ammonium and a nitrate of an alkaline metal intimately mixed and which by double decomposition produces a vapor of alkaline metal chlorid sufficient to damp the flame to prevent ignition and explosion of coal dust laden atmosphere and of fire damp.

4. A detonating explosive containing a mixture of a chlorid, and a nitrate of a metal of the alkalies intimately mixed which on explosion will produce a vapor of a chlorid of the metal of the alkalies sufficient to damp the flame, and prevent the ignition of coal-dust laden atmosphere and fire damp.

5. A short flame detonating explosive containing substantially combining weights of ammonium chlorid and a nitrate of a metal of the alkalies intimately mixed in proportions sufficient to dampen the flame and prevent the ignition of coal dust laden atmosphere and fire-damp.

6. A short flame detonating explosive containing substantially combining weights of ammonium chlorid and sodium nitrate intimately mixed in proportions sufficient to dampen the flame and prevent the ignition of coal dust laden atmosphere and fire-damp.

7. A short flame detonating explosive containing about ten per cent. of a mixture of ammonium chlorid and sodium nitrate said substances being present in the proportion of their combining weights.

In testimony that I claim the foregoing as my invention, I have signed my name in presence of two subscribing witnesses.

CHRISTIAN EMIL BICHEL.

Witnesses:

MAX KAEMPFF,  
ERNEST H. L. MUMMENHOFF.